

2,857,258

## JET PROPELLANT

Charles A. Thomas, Dayton, Ohio, assignor to Monsanto Chemical Company, St. Louis, Mo., a corporation of Delaware

No Drawing. Application August 22, 1945  
Serial No. 612,133

6 Claims. (Cl. 52—5)

The present invention relates generally to impulse generating compositions and more particularly to compositions suitable for the production of a high velocity gas jet, the reactive impulse of which may be employed to perform useful work such as the propulsion of rocket shells (including anti-aircraft or anti-tank projectiles) or in assisting the take-off of airplanes, gliders, accelerating the movement of wheeled vehicles, etc.

Compositions of the type described herein are generally employed as a gas generating fuel in a chamber referred to herein as a "motor" and which usually consists of a cylindrical fuel chamber closed at one end and provided at the opposite end with a coaxial orifice or throat of the Venturi type. The chamber is so constructed as to be capable of withstanding the high gas pressure which is developed by combustion of the fuel. The products of combustion of the fuel issue as a high velocity gas jet through the throat of the motor, the reactive effect of the gas creating the propelling impulse employed in rocket or jet propulsion.

When motors of the foregoing type are employed in the propulsion of artillery shells such as anti-tank or anti-aircraft shells the motor containing the propellant is generally attached to the base of the shell, the whole assembly being fired from a smooth bore tube or rack. For use in assisting the take off of aircraft or accelerating the motion of vehicles generally, one or more of the motors may be mounted upon the plane or vehicle in such a way that the impulse created by the high velocity gas jet is transmitted directly to the aircraft or vehicle.

The present compositions are adaptable to a wide variety of purposes, depending upon the rapidity and conditions under which they are burned. They may be adapted to the propulsion of artillery shells, in which case the burning time is relatively short. They may also be adapted for assisting the take-off of airplanes either from land or water, in which case the burning time is considerably lengthened. In other cases they may be used to assist in starting or accelerating the motion of vehicles such as railroad trains, in which case the burning time is still somewhat longer. By a suitable variation in the composition, as will be hereinafter more fully described, impulse generating compositions suitable for these various purposes may be produced.

In determining the suitability of any gas generating composition for impulse, rocket or jet propulsion purposes, the most important properties of the fuel to be considered are: (1) its specific impulse, (2) the reproducibility of its burning properties, and (3) the relation between its rate of burning, the pressure and the temperature. The specific impulse is the total impulse (i. e., force-time integral) imparted to the motor per unit weight of propellant consumed and provides a measure of the performance to be expected from a motor or rocket using the fuel in question. Reproducibility is indispensable if power and freedom from bursts are to be obtained; while a low dependence of rate of burning on pressure and preignition temperature greatly sim-

plifies motor design, increases the range of climatic conditions under which the device is usable and decreases the hazards which arise from small variations in the property of the fuel.

5 The foregoing critical properties are all fundamentally related to the rate of burning of the fuel and this, in turn is known to be dependent upon (1) the burning area of the fuel, (2) the pressure within the motor and (3) the pre-ignition temperature of the fuel. Considering firstly the burning area factor, it is known that the rate of burning will vary if the burning area of the fuel as it is consumed is either decreasing (called a "degressive" or "regressive" burning area) or increasing (called a "progressive" burning area). The effect of 10 this factor may be minimized to a considerable extent by forming the composition into bodies (called "grains") having geometric forms so designed and inhibited as to insure a substantially constant burning area as the fuel is consumed.

20 Considering now the effect of pressure on the burning rate, from theoretical considerations, it will be apparent that when the fuel is ignited, the pressure within the motor chamber rises from atmospheric pressure to a higher pressure at a steady state. Inasmuch as the 25 pressure existing within the rocket motor greatly affects the burning rate, erratic behavior likely to result in explosions of the fuel chamber may be anticipated if the fuel is characterized by a pronounced dependence of burning rate upon pressure. Considering the burning phenomena in greater details, after ignition of the fuel, the pressure within the motor chamber will rise until the 30 rate of gas formation within the chamber equals the rate of efflux, at which point a "steady condition" will be attained. Since the rate of gaseous combustion products is proportional to the burning area of the grain ( $A_g$ ) and also to some power of the pressure ( $P^n$ ) and since the rate of efflux is proportional to the pressure  $P$  and to the area of the orifice or throat ( $A_t$ ) a "steady state" will exist when:

$$40 \quad K_1 A_g P^n = K_2 A_t P$$

the "steady state pressure" is therefore given by:

$$P \propto \left( \frac{A_g}{A_t} \right)^{1/(1-n)}$$

45 provided  $n$  is less than unity.

The foregoing relation (the so-called "burning law" in one of its various forms) is an exceedingly important relation in the study of fuels suitable for rocket purposes. By assuming that the "steady state" pressure is 50 equal to the maximum pressure produced in the rocket motor ( $P_m$ ) the relation becomes:

$$P_m \propto \left( \frac{A_g}{A_t} \right)^{1/(1-n)}$$

55 since  $P_m$ ,  $A_g$  and  $A_t$  are all readily measurable quantities, it is possible to plot  $\log P_m$  against  $\log (A_g/A_t)$ . Such a plot will describe a straight line of the slope-intercept form, the slope of the line being the exponent  $1/(1-n)$ , from which the value of the exponential constant  $n$  may be determined.

In the case of actual propellants, some deviation from the so-called "burning law" may be observed. However, the smaller the average deviation of the observed pressures from a smooth plot of pressure against  $A_g/A_t$ , the 65 more highly reproducible will be the internal ballistics of the fuel. Moreover, the closer the value of  $n$  approaches zero, the less sensitive does the system become to small variations in  $A_g$  and  $A_t$ ; i. e., the less rapidly will the pressure vary with small variations in the conditions of burning such as the grain area, obstructions in the throat of the motor, etc. Conversely, the closer

the value of  $n$  approaches unit, the more sensitive does the system become to variations in grain area and throat area, and in the limiting case where  $n$  becomes unity, it will be apparent that the pressure varies as the infinite power of the  $A_g$  to  $A_t$  ratio.

Thus the so-called "burning law," and particularly the value of  $n$ , the exponential constant, are of fundamental importance in the selection of a rocket propellant and in the design of the rocket motor; a fuel that deviates only slightly from the so-called "burning law" and that possesses a low value of  $n$  will be characterized by a high reproducibility of chamber pressures, thereby permitting the use of lighter chamber walls and generally of a lower factor of safety in motor design.

Turning now to the effect of temperature on the burning rate, a low dependence of the burning rate on the temperature of the fuel prior to ignition (referred to as "ambient" or "pre-ignition" temperature) is of the utmost importance in rocket design, for several reasons. In the first place, if the fuel has a large temperature coefficient of pressure (i. e., rate of change of pressure with respect to pre-ignition temperature, in a given motor using a grain of given area  $A_g$ ), a motor that is safe to use at low pre-ignition temperatures may burst if used, for example, under hot desert conditions. On the other hand, if the motor is designed for use at high pre-ignition temperatures, then it is unnecessarily massive for use under moderate or low temperature conditions. Furthermore, if the pressure developed in the rocket motor falls below a certain threshold value, the propellant tends to burn incompletely. Therefore, if the fuel is characterized by a large temperature coefficient, the possibility is increased of "burn-outs" at low pre-ignition temperatures, as well as "blow-outs" at high pre-ignition temperatures. Finally, a fuel with a large temperature coefficient will be characterized by an undesirably high degree of dispersion at low pre-ignition temperatures, and also by variable ballistics (changes in range) with variations in the temperature of the fuel prior to ignition.

Considering the temperature factor somewhat more closely, it has been found that, if the rate of burning is measured at different ambient temperatures but at the same maximum pressure, then the rate of change of burning with temperature is relatively small in the case of practically all existing rocket fuels. Unfortunately, however, in actual use, the only factor capable of being maintained substantially constant is the ratio:  $A_g/A_t$ , i. e., the grain area and the throat area. In other words, the maximum pressure developed in the motor chamber is not a constant but varies with the ambient temperature. But as previously explained, in the case of fuels having a large value of  $n$ , changes in pressure profoundly affect the rate of burning. Accordingly, the temperature effect is intimately related to the pressure effect.

The temperature effect discussed above is more precisely defined by the relation:

$$\frac{1}{P} \left( \frac{dP}{dT} \right) K = \frac{1}{R} \left( \frac{dR}{dT} \right) K = \frac{1}{R} \left( \frac{dR}{dT} \right) P$$

where  $P$  is the pressure,  $T$  is the temperature,  $R$  is the rate of burning,  $K$  is a constant  $A_g/A_t$  ratio, and  $n$  is the exponential constant in the so-called "burning law." Expressing the same relation in words, the fractional rate of change of pressure with temperature for a grain of given area  $A_g$  when burned in a motor having a throat area  $A_t$ , is equal to the fractional change in the burning rate at a constant  $A_g$  to  $A_t$  ratio, and this, in turn, is equal to the fractional change in the burning rate at constant pressure, divided by  $1-n$ . Therefore, the smaller the value of the exponential constant  $n$ , the smaller will be the temperature coefficient of the rate of burning at a constant  $A_g$  to  $A_t$  ratio. Conversely, if  $n$  approaches unity, the temperature coefficient of the burning rate at a constant  $A_g$  to  $A_t$  ratio approaches infinity.

From the foregoing, it will be apparent that a small value of the exponential constant  $n$  in the so-called "burning law" is of the utmost significance in the design of an impulse motor for use with a selected fuel. Moreover, it will be evident that, inasmuch as the constant  $n$  is an exponential factor, a fuel which has an  $n$  value of, say, 0.5 performs in a radically different manner from one whose  $n$  value is, say, 0.666, even though the difference in the  $n$  values may appear to be numerically very small. Thus, since the ratio  $A_g/A_t$  is usually a large number (e. g., 200) the difference between

$$\left( \frac{A_g}{A_t} \right)^{1/(1-0.5)}$$

and

$$\left( \frac{A_g}{A_t} \right)^{(1/1-0.666)}$$

is the difference between the square and cube of a very large number; for instance, the difference between  $(200)^2$  and  $(200)^3$  which in this case amounts to 7,960,000. Small numerical differences in  $n$  values of impulse fuels are, accordingly, of great significance, not only in respect to reproducibility at a substantially constant pre-ignition temperature, but also with respect to uniformity of action under varying pre-ignition temperatures.

In the preceding paragraphs, the importance of (1) a small deviation from the "burning law," (2) a small  $n$  value, and (3) a low-temperature coefficient, have been discussed. In addition to these factors, it is also desirable to employ a propellant characterized by as high a density as possible, inasmuch as a high density permits the use of a smaller firing chamber, thereby making it possible to decrease the size and mass of the motor and therefore to improve the ballistics of the motor.

From the above analysis it will be apparent that the design of the impulse fuel presents an exceedingly complex problem, the solution of which is complicated by the fact that the properties of a gas generating composition under atmospheric conditions afford practically no indication of the properties of such composition when burned under the conditions obtaining in an impulse motor. In short, the design of a propellant fuel for jet propulsion at the present time is almost entirely an empirical problem that requires the most painstaking and protracted experimentation.

Broadly speaking, the object of the present invention is to provide a new and improved gas generating composition suitable for rocket purposes.

A more particular object is the provision of a novel impulse propellant characterized by:

- (1) A burning rate which deviates only slightly from the so-called "burning law";
- (2) A low value of the exponential constant  $n$  in the "burning law";
- (3) A low temperature coefficient of pressure change when a fuel of given grain area is fired in a given motor at various pre-ignition temperatures.

A further object is a propellant possessing the following additional characteristics:

- (a) A sufficiently high specific impulse;
- (b) Relatively constant external ballistics;
- (c) A burning rate which may be made high or low at will;
- (d) Adaptability to the production of grains of high and low burning times;
- (e) High mechanical strength and freedom from distortion under stress;
- (f) High loading density;
- (g) Moderate motor chamber requirements;
- (h) Adaptability to molding to close dimensional tolerances without mechanical finishing operations;
- (i) Ready availability of raw materials;
- (j) Relative simplicity of the equipment required for fabrication.

Other objects and advantages will become apparent as the invention is hereinafter more particularly described.

As the result of an extended investigation it has been found that the objects set forth above may be obtained by a novel type of propellant consisting of a particulate gas generating composition compacted in the presence of a binder comprising a chlorinated polyphenyl body. More particularly, the gas generating composition herein provided consists essentially of two components; namely, (1) a particulate non-plastic gas generating composition and (2) a binder comprising a resinous chlorinated diphenyl or terphenyl with or without one or more resinous bodies. Propellants of the present type differ fundamentally from previous fuels of the smokeless powder (ballistite) type wherein the plastic component of the composition was a major constituent. In the composite fuels of the present invention the solid non-plastic gas generating component constitutes generally as high as 90-95% of the composition, the plastic component being employed in relatively small proportions which serves not only as a binder but as a modifier of the burning characteristics of the gas generating component.

### I. THE GAS GENERATING COMPONENT

The gas generating component in accordance with the present invention consists of a mixture of finely divided solid materials which are capable of interaction under the influence of heat to produce a large volume of gaseous reaction products. Mixtures of this type usually consists of an oxidizing substance and an oxidizable substance. The oxidizing substance may comprise one or more solid inorganic oxidizing agents such as the nitrates, for example, sodium nitrate, potassium nitrate, barium nitrate, ammonium nitrate and the like. The oxidizable substance desirably comprises one or more solid organic nitro compounds or their salts, such as the sodium or preferably the ammonium salts of nitro phenols (for example, ammonium picrate) or one or more solid nitramines (for example, nitroguanidine).

In general, the oxidizable substance and the oxidizing substance may be employed in a wide range of proportions, depending on the particular use to which the ultimate fuel is to be put. In some instances, it may be desirable to use the components in the proportions required for oxygen balance for the production of  $\text{CO}_2$  and  $\text{H}_2\text{O}$  (i. e., zero oxygen balance); in the case of ammonium picrate=sodium nitrate mixtures this result is obtained with a weight ratio of 52.5 to 47.5, respectively. However, for other purposes, a different specific impulse or a different burning rate may be desirable, in which case the relative proportions of components may be considerably altered with a view to modifying one or more properties of the fuel. Thus, for aircraft take-off purposes or for other uses where a low rate of burning is desirable, a 10-90 sodium nitrate=ammonium picrate composition may be satisfactory, whereas for anti-aircraft rockets or other purposes where a high rate of burning is desirable a 50-50 mixture of these same components may be preferable.

Generally speaking, in the case of ammonium picrate-potassium nitrate mixtures, it is undesirable to employ in excess of about 55% potassium nitrate, since a further increase in this component increases the solid reaction product (potassium carbonate) at the expense of the gaseous products, thereby cutting down the power of the propellant. A high specific impulse will be obtained with mixtures containing from about 10% to about 55% potassium nitrate. A high rate of burning will be obtained with a composition containing ammonium picrate 45%, potassium nitrate 55%.

Certain general principles governing the relation of composition to impulse are reasonably clear. Any change in composition which lowers the proportion of solid reaction product tends to increase the specific impulse, in any case more than compensating for an accompanying

decrease in heat of reaction. Thus, an increase in the proportion of ammonium picrate in a mixture with potassium nitrate beyond the 48.5% required for a zero oxygen balance leads to a decrease in the predicted heat of reaction. Nevertheless, the specific impulse increases slightly. On the other hand, increase in the proportion of potassium nitrate beyond 55% produces a marked decrease in specific impulse. In this case the increase in proportion of potassium oxide or potassium carbonate formed works in the same direction as the decrease in heat of reaction. Generally speaking, the specific impulse of a propellant producing upon combustion solid as well as gaseous reaction products, is related to the fraction of gaseous product, the heat of reaction, the mean molecular weight and the heat capacity of the gaseous product. This general observation serves as a useful guide in devising new proportions of ingredients.

In some cases, it may be desirable to incorporate small amounts of other materials in the gas generating composition, in order to modify one or more characteristics of the molding powder or of the finished propellant. Thus, a small amount of a readily combustible material such as aluminum powder, charcoal, sulfur and the like, may be added for the purpose of modifying the burning properties of the fuel.

### II. THE BINDER

The chlorinated polyphenyl products mentioned above, which may be used as binders in accordance with the present invention, may comprise the chlorinated diphenyls or chlorinated terphenyls and mixtures thereof. Chlorinated polyphenyls suitable as binders for the production of the composite gas generating body may be prepared as described by Jenkins et al., in United States Patent 1,892,400. When diphenyl, alone, is chlorinated, the chlorine content should be at least 54% by weight and may be as high as 64% or 65% by weight. These products are preferably used in the non-crystalline form as described in the above patent; however, some crystalline phase resulting from a somewhat higher degree of chlorination may also be present. As described in the above mentioned Jenkins et al. patent some higher boiling aromatic hydrocarbons related to diphenyl (and comprising the terphenyls) may also be present in the material undergoing chlorination. As a matter of fact, for the present purpose, the binder may comprise wholly the chlorinated terphenyl fraction, but generally it appears desirable to employ a mixture of diphenyl and terphenyl as the hydrocarbon which is chlorinated, to the extent of between 40% and 60% or 65% by weight of chlorine. For the purpose of the present specification and claims, the chlorinated diphenyl and/or terphenyl product is referred to as chlorinated polyphenyl.

While the chlorinated diphenyls and/or terphenyls may be used alone as the binder and burning rate modifier, for certain purposes it may be desirable to incorporate additional resinous compounds therewith for the purpose of increasing the tack and strength of the binder. For this purpose, I may use any resinous materials such as phenol-formaldehyde or urea-formaldehyde resins. The phenolic constituent of these phenol-formaldehyde resins may be ordinary phenol, cresol, para-phenyl phenol or tertiary butyl phenol. These resins are employed in the heat-reactive condition so that upon heating, which may take place at a lower temperature, they become infusible and insoluble. When oil-soluble phenolic resins such as the para-phenyl phenol-formaldehyde or tertiary butyl phenol-formaldehyde resins are employed, the binder may include a solvent for these resins. These solvents may be drying oil such as tung or linseed oil. Phenol-formaldehyde resins in the "B" stage are soluble in alcohol and may be added while dissolved in this type of solvent. On the other hand, urea-formaldehyde resins in the heat-

reactive state may be employed as solutions in toluene, xylene and butanol. These resins may be prepared as described in United States Patent No. 2,171,882, issued September 5, 1939.

The binder is incorporated into the gas generating composition by simple mixing with the gas forming materials. If the mixture of gas forming material and binder is rolled upon slightly heated rolls for a few minutes, a more intimate mixing of the ingredients is obtained. Where a solvent is present in the binder composition, the material may also be rolled upon cold rolls. Pigment rolls such as are employed in the paint industry may be used. During rolling, any solvent present in the resinous binder is readily evaporated and the operation of rolling desirably should be continued until a dry, powdery material free of solvent is obtained.

In order to avoid adversely affecting the internal ballistics of the propellant, a restricted amount of resinous binder should be employed; namely, an amount of resin merely sufficient to enable the production of the mechanically strong grain to be achieved. Usually from 5% to 10% by weight of resin in the finished grain is sufficient to obtain the desired mechanical properties without adversely affecting the burning characteristics of the composition. In some cases, as little as 3% of resin as binder may be satisfactory.

### III. COMPOUNDING THE INGREDIENTS

In producing the composite propellant of the present invention the oxidizing component (for example, potassium nitrate) is preferably first dried and then ground to a finely divided condition. The powdered oxidizable component (for example, ammonium picrate) is mixed with the oxidizing agent, the former likewise being in a finely powdered condition. The chlorinated polyphenyl binder with or without a resinous binder is next added and thoroughly incorporated therewith. As stated above, if the mixture be rolled upon heated rolls, the temperature of which is just sufficient to soften the binder, more intimate mixing is achieved. Where a resinous binder is employed in conjunction with a thermostating resin, the rolling operation serves not only to more intimately mix together the ingredients but also permits any solvent present to evaporate.

The mixed powder so obtained is pressed in a die under sufficient pressure to produce a dense pellet or grain. After pressing the grain, if a thermosetting resin has been employed as a constituent of the binder, the grain is desirably cured at a temperature sufficient to render the resin insoluble and infusible. Temperatures between 30° C. and 80° C. may be employed for curing the resin. Condensation catalysts may be present in the composition in order to accelerate the curing reactions.

### IV. CEMENTING AND COATING THE GRAINS

Because of the powdery nature of the composition resulting from the incorporation of the resinous binder with the solid gas generating ingredients an inherently high degree of internal friction in the pressing operation renders it difficult to mold very low grains. Where such long grains are desired, a plurality of short, readily molded grains may be cemented together by means of any suitable cement containing thermosetting resins such as alkyd resins, etc., the resulting composite fabricated grains exhibiting excellent properties, as will be herein-after described.

For many jet propulsion applications it is of considerable advantage to be able to restrict the burning of the fuel body to certain parts of its surface, either for the purpose of producing a grain of neutral burning area, or for the purpose of restricting the burning of the grain to a particular area of the grain. The compositions of the

present invention are particularly adapted to the formation of such "restricted burning grains" inasmuch as the binder will not diffuse into and adversely affect coating materials designed to prevent burning on certain parts of the surface.

As the result of an extensive survey, it has been found that practically any standard varnish or paint containing either a drying oil such as linseed oil or an alkyd resin produces an excellent flame-resisting coating. Thus a large variety of paints and varnishes including standard spar varnish, automobile paint, barn and roof paint, asphalt varnish and many other types of available coating material may be used as flame-resisting coatings. The coating materials may be conveniently applied to the grains by painting, spraying or dipping, followed by drying in any manner suited to the character of the applied coating. Thereafter the coated surface may be additionally protected by means of adhesive textile tapes or by other suitable means. Such coatings have been found to withstand pressures well over 2,000 lbs./in.<sup>2</sup>.

### V. EXAMPLE

In order more clearly to disclose the nature of the present invention, a preferred embodiment will now be described in considerable detail. It should be clearly understood, however, that this is done solely for the purpose of illustrating the principle of the invention by means of a concrete example. Accordingly, the following detailed description is not to be construed as a limitation upon the spirit or scope of the invention which is more particularly defined in the appended claims.

In producing the preferred gas generating composition of the present invention, commercially pure potassium nitrate is first dried to less than 1/10% of water, then ground to a particle size preferably to 70% minus 325 mesh standard screen size. The dry, powdered potassium nitrate is thoroughly mixed with finely precipitated ammonium picrate in the proportion of 55:45 by weight.

A non-crystalline, chlorinated polyphenyl resin such as is described in Example VI of United States Patent 1,892,400 in powdered form is mixed therewith in the proportions of 90 parts by weight of the potassium nitrate-ammonium picrate mixture to 10 parts by weight of chlorinated polyphenyl resin. The powdery mixture is then incorporated on heated rolls for a few minutes. At the completion of rolling, the material is allowed to cool and then again finely powdered. The powder so produced is formed into a grain by pressing in a heated die.

The grains are now ready for use either as formed or after cementing several grains together to form a larger grain or after coating with a flame-resisting material to form "restricted burning grains." Cementing may be conveniently carried out by applying a thin coat of cement (alkyd resins such as Glyptal 1201) to the surfaces to be joined, pressing the two surfaces together and maintaining a light pressure on the joined portions during the curing operation. Restricted burning grains may be produced by spraying a selected area such as the ends of a perforated cylindrical grain if neutral burning is required, or the sides and one end of a large, solid, cylindrical grain with any commercial coating material containing linseed oil or an alkyd resin. The coated surface may be additionally protected by applying an adhesive coated fabric tape over the resin coating.

### VI. PROPERTIES OF THE COMPOSITE PROPELLANT

Table I summarizes the ballistically important properties of the two specific compositions in accordance with the present invention. For purposes of comparison the corresponding data on ballistite are also given.

9  
Table I

|                                                    | Ballistite | C. P.-1 <sup>1</sup> | C. P.-2 <sup>2</sup> |
|----------------------------------------------------|------------|----------------------|----------------------|
| Density, g./cc.                                    | 1.63       | 1.92                 | 1.79                 |
| $dl/dT$ (Burning rate at 2,000 p. s. i., in./sec.) | 1.00       | 1.40                 | 1.42                 |
| $dlnP/dT = (dlnR/dT)K$                             | 1.5%       | 0.5%                 | 0.5%                 |
| Exponential Constant $n$                           | 0.73       | 0.40                 | 0.40                 |
| $K_{2000} = (A_g/A_t)_{2000}$                      | 200        | 220                  | 220                  |
| $I_{2000}$                                         | 226        | 165                  | 170                  |

<sup>1</sup> The composition listed as C. P.-1, contained the following ingredients in percent by weight: 45% NaNO<sub>3</sub>, 45% ammonium picrate and 10% of a chlorinated diphenyl-polyphenyl resin.

<sup>2</sup> The composition listed as C. P.-2, contained the following ingredients in percent by weight: 47% NaNO<sub>3</sub>, 47% ammonium picrate, 4.3% of a urea-formaldehyde resin and 1.7% of a chlorinated diphenyl resin.

From the foregoing data it will be apparent that the composite propellant of the present invention is characterized by the following advantageous properties:

(1) The material has highly reproducible ballistics. The logarithmic plot of pressures against  $A_g/A_t$  is a straight line over the range of from 1,000 to 4,000 p. s. i.

(2) The linear rate of burning of the present fuels can be varied over a wide range. This may be accomplished by changing either the specific composition of the powdery gas generating composition or the specific composition of the binder. Thus, the present propellant lends itself to a wide variety of uses requiring entirely different burning rates.

(3) The rate of burning has a low dependence on pressure. The exponential constant  $n$  in the "burning law" has a value of about 0.4 to about 0.5, depending on the composition over a pressure range of from 500 to 14,000 p. s. i. for grains of neutral burning area. From this it follows that the pressure in the rocket motor will vary as the 1.7 power of the  $A_g$  to  $A_t$  ratio. For comparison, the value of  $n$  for smokeless powder is about 0.7 and the area-pressure exponent is about 3.7. Because of the low value of  $n$  for the composite propellant of the present invention, a much smaller change in chamber pressure will result from any irregularity in burning which causes a change in the burning area or from variations in orifice or throat area. Furthermore, the low  $n$  value insures a lower pressure drop along a long grain than in the case of smokeless powder. Together with the high reproducibility of the chamber pressure, it permits the use of lighter chamber walls and generally a lower factor of safety in motor design.

(4) The rate of burning has a low dependence on temperature. In the case of the present fuels, over the range from -40 to +60° C., the pressure increases only about 0.50% for each degree centigrade rise in temperature. For smokeless powder the corresponding figure appears to be of the order of 15%, per 10° C.

(5) The value of  $K$  (i. e.,  $A_g$  to  $A_t$  ratio) may be varied over a wide range. This may be accomplished by modifying the specific composition of the grain.

(6) The specific impulse is satisfactorily high (of the order of 160-170 for optimum expansion ratio).

(7) The composite propellant has a high density (e. g., about 1.75 to 1.85 grams per cc.), which permits an appreciably higher load density than with smokeless powder (density about 1.63 grams per cc.). In addition, the low values of  $n$  and  $K$  (see items 2 and 4) permit the use of smaller port areas in the motor chamber and this also favors high loading density.

(8) The composite propellant has a high crushing strength (about 5,000 to 12,000 p. s. i. depending on the composition) and suffers no significant distortion under stresses short of those required for fracture.

(9) It may be molded to close dimensional tolerances and requires no substantial amount of finishing by machining operations.

(10) The impact sensitivity of the material is satis-

## 10

factory (approximately the same as that for ammonium picrate).

(11) The chemical stability of the material is satisfactory as judged by the usual accelerated tests. The ballistic properties of grains burned after storage for several months have been satisfactory in that no change has taken place. Many grains have been subjected to a temperature cycle of 8 hours per cycle between +60° C. and -45° C. for 20 cycles without showing any significant change in ballistic properties, in density, or in compression strength.

(12) The burning of the cemented grains shows no irregularities whatever arising from the composite, built-up or fabricated structure.

(13) The restriction of the burning area by means of protective coatings is entirely successful. The grains contain no diffusible liquid, such as nitroglycerine, which has caused so much trouble in attempts to restrict burning of double base powder grains.

20 What I claim is:

1. A composite jet propulsion propellant essentially composed of a dense, compact mixture of crystalline particles of ammonium picrate and particles of a crystalline inorganic nitrate selected from the class consisting of 25 sodium nitrate, potassium nitrate, barium nitrate and ammonium nitrate, said mixture containing between 10% and 55% of said nitrate, the balance of said mixture being particles of ammonium picrate and from 5% to 10% of a resinous matrix for said particles, said matrix consisting of a material selected from the class consisting of resinous chlorinated polyphenyls containing at least 40% of chlorine and mixtures of chlorinated polyphenyls containing at least 40% chlorine with a urea-formaldehyde resin.

35 2. A composite jet propulsion propellant essentially composed of a dense, compact mixture of crystalline particles of ammonium picrate and potassium nitrate, said mixture containing between 10% and 55% of said nitrate and the balance thereof being ammonium picrate and from 5% to 10% of said mixture of a resinous matrix for said particles, said matrix consisting of a chlorinated polyphenyl containing between 42% and 65% by weight of chlorine.

45 3. A composite jet propulsion propellant essentially composed of a dense, compact mixture of crystalline particles of ammonium picrate and potassium nitrate, said mixture containing between 10% and 55% of said nitrate and the balance thereof being ammonium picrate and from 5% to 10% of said mixture of a resinous matrix for said particles, said matrix consisting of a chlorinated polyphenyl resin containing between 42% and 65% by weight of chlorine, said propellant having a density of 50 1.92.

55 4. A composite jet propulsion propellant essentially composed of a dense, compact mixture of crystalline particles of ammonium picrate and potassium nitrate, said mixture containing between 10% and 55% of said nitrate and the balance thereof being ammonium picrate and from 5% to 10% of said mixture of a resinous matrix for said particles, said matrix consisting of a mixture of a urea-formaldehyde resin and a chlorinated polyphenyl resin containing between 42% and 65% by weight of chlorine, said propellant having a density of 60 1.79.

65 5. A composite jet propulsion propellant essentially composed of a dense, compact mixture of crystalline particles of ammonium picrate and sodium nitrate, said mixture containing 45% sodium nitrate, 45% of ammonium picrate and a resinous matrix for said particles, said matrix consisting of 10% of a chlorinated polyphenyl resin containing between 42% and 65% of chlorine.

70 6. A composite jet propulsion propellant essentially composed of a dense, compact mixture of crystalline particles of ammonium picrate and sodium nitrate, said mixture containing 47% of sodium nitrate and 47% of ammonium picrate and a resinous matrix for said parti-

cles; said matrix consisting of 41.3% of a urea-formaldehyde resin and 1.7% of a chlorinated polyphenyl resin containing between 42% and 65% of chlorine.

References Cited in the file of this patent

UNITED STATES PATENTS

|           |         |               |
|-----------|---------|---------------|
| 363,224   | Gerhard | May 17, 1887  |
| 1,892,400 | Jenkins | Dec. 27, 1932 |
| 1,975,072 | Booth   | Oct. 2, 1934  |
| 2,159,234 | Taylor  | May 23, 1939  |
| 2,165,263 | Holm    | July 11, 1939 |
| 2,195,965 | Holm    | Apr. 2, 1940  |
| 2,365,170 | Bitting | Dec. 19, 1944 |

5

|           |
|-----------|
| 2,409,111 |
| 2,433,417 |
| 2,434,872 |

|                |               |
|----------------|---------------|
| Davis          | Oct. 8, 1946  |
| Bitting et al. | Dec. 30, 1947 |
| Taylor         | Jan. 20, 1948 |

FOREIGN PATENTS

|               |              |
|---------------|--------------|
| Great Britain | A. D. 1888   |
| Great Britain | A. D. 1892   |
| Great Britain | A. D. 1899   |
| Great Britain | A. D. 1905   |
| Germany       | July 4, 1921 |

OTHER REFERENCES

Penning, "Chlorinated Diphenyl," Ind. and Eng. Chem., November 1930, pages 1180 and 1182.

UNITED STATES PATENT OFFICE  
CERTIFICATE OF CORRECTION

Patent No. 2,857,258

October 21, 1958

Charles A. Thomas

It is hereby certified that error appears in the printed specification of the above numbered patent requiring correction and that the said Letters Patent should read as corrected below.

Column 1, line 70, and column 2, line 28, for "depedence", each occurrence, read -- dependence --; column 3, line 1, for "unit" read -- unity --; column 7, line 42, for "thermostating" read --thermosetting--; line 62, for "low" read -- long --.

Signed and sealed this 31st day of May 1960.

SEAL)

Attest:

EARL H. AXLINE  
Attesting Officer

ROBERT C. WATSON  
Commissioner of Patents